

## UNITED STATES PATENT OFFICE

2,446,207

FROTH FLOTATION OF ORES EMPLOYING A  
WATER-SOLUBLE SALT OF A CYMENE  
SULFONIC ACIDWilliam T. Bishop, Wilmington, Del., assignor to  
Hercules Powder Company, Wilmington, Del.,  
a corporation of DelawareNo Drawing. Application April 11, 1945,  
Serial No. 587,833

7 Claims. (Cl. 209—166)

1

This invention relates to a process for concentrating ores and more particularly to a froth flotation process in the presence of cymene sulfonates.

Various sulfates and sulfonates of organic compounds, such as sulfonated castor oil, alkyl-substituted naphthalene sulfonated acids, and sulfuric acid esters of normal primary alcohols having from 6 to 18 carbon atoms have been suggested as flotation reagents. Many of these, in addition to producing froths, also show some collecting properties for several minerals. This is a disadvantage because it results in poor selectivity of the mineral over the gangue in the ore. These sulfates and sulfonates usually produce a froth composed of large bubbles which collapse under the weight of the mineral film. The vol-

2

was retained by an 8-mesh screen, was ground for 15 minutes in a ball mill with 3 lbs. of lime per ton of ore and 1000 cc. of water. The ore contained the minerals, chalcopyrite, chalcocite, pyrite, covellite, and bornite; the gangue materials were chiefly feldspar and sericite. The ground ore was screened through a 48-mesh screen and transferred to a 1000 g. flotation machine. The pulp was conditioned for 10 minutes with 0.04 lb. potassium cyanide per ton of ore. Water was added to dilute the pulp to about 20% solids. The frother reagent given in Table 1 was added and a sodium dithiophosphate (Aerofloat) type collector was added in an amount equal to 0.08 lb. per ton of ore. Air was drawn through the pulp and a concentrate was scraped off for 10 minutes. The results are given in Table 1.

Table 1

| Example | Frother Reagent                                                              | Lb. per Ton         | Copper in Tailings | Copper in Concentrate | Copper Recovery |
|---------|------------------------------------------------------------------------------|---------------------|--------------------|-----------------------|-----------------|
| 1.....  | p-Cymene sodium sulfonate (about 30% inorganics).....                        | 0.30                | Per cent<br>0.16   | Per cent<br>27.8      | Per cent<br>82  |
| 2.....  | {p-Cymene sodium sulfonate (about 30% inorganics).....<br>Cresylic acid..... | 0.18<br>0.09 } 0.15 |                    | 27.2                  | 84              |

ume of the froth is difficult to control. Immediately after the addition of the frothing agent, a voluminous froth is produced which has a short cell life. The prior art sulfates and sulfonates cause some gangue minerals to be floated and thus result in a low grade concentrate.

It has been found that the above disadvantages are overcome by the use of a water-soluble salt of cymene sulfonic acid as a flotation agent. These reagents function as frothers and do not show any collection properties, thus, bringing about a clean separation. The characteristics of the froth produced are ideal for mineral flotation. The bubbles produced are small and the froth has a long cell life. The reagents have marked selectivity and the amount of gangue minerals floated is small. A high grade concentrate is obtained.

The process of this invention is illustrated by the following examples.

## EXAMPLES 1-2

A 1010 g. sample of a copper sulfide ore, which 50

was retained by an 8-mesh screen, was ground for 15 minutes in a ball mill with 1000 cc. of water. The ore contained the minerals, chalcopyrite, chalcocite, pyrite, covellite, and bornite; the gangue materials were chiefly feldspar and sericite. The ground ore was screened through a 48-mesh screen and transferred to a 1000 g. flotation machine. The pulp was conditioned for 10 minutes with 0.04 lb. potassium cyanide per ton of ore. Water was added to dilute the pulp to about 20% solids. The frother reagent given in Table 1 was added and a sodium dithiophosphate (Aerofloat) type collector was added in an amount equal to 0.08 lb. per ton of ore. Air was drawn through the pulp and a concentrate was scraped off for 10 minutes. The results are given in Table 1.

## EXAMPLES 3-4

A 1010 g. sample of the copper sulfide ore, described in Examples 1-2, which was retained on an 8-mesh screen, was ground for 15 minutes in a ball mill with 1000 cc. of water. The ground ore was screened through a 48-mesh screen and transferred to a 1000 g. flotation machine. To this was added 2.0 lbs. of lime per ton of ore, 0.04 lb. potassium cyanide per ton of ore, 0.06 lb. Aerofloat No. 25 per ton of ore, and the frother as given in Table 2. All were conditioned with the ore for 10 minutes. Then air was drawn through the pulp and a concentrate was scraped

off for 10 minutes. The results are given in Table 2.

the tailings, a high grade concentrate and a relatively high recovery.

Table 2

| Example | Frother Reagent                                    | Lb. per Ton | Copper in Tailings | Copper in Concentrate | Copper Recovery |
|---------|----------------------------------------------------|-------------|--------------------|-----------------------|-----------------|
| 3.....  | p-Cymene calcium sulfonate.....                    | 0.24        | Per cent<br>0.25   | Per cent<br>21.7      | Per cent<br>73  |
| 4.....  | p-Cymene sodium sulfonate (18-20% inorganics)..... | 0.24        | 0.26               | 19.7                  | 71              |

The p-cymene calcium sulfonate was prepared by the following method: fifty grams of p-cymene was added slowly to 52.7 g. of oleum at 20-30° C. The mixture was agitated at a temperature of 50° C. for 4 hours. The product was added to 200 g. of ice and then neutralized with excess calcium carbonate and the precipitated calcium sulfate and excess calcium carbonate were removed by filtration. The filtrate was evaporated to dryness to recover the p-cymene calcium sulfonate.

## EXAMPLES 5-6

A flotation pulp of a lead sulfide ore, which is composed of galena with small amounts of pyrite in a dolomite gangue was prepared. A volume of this flotation pulp, corresponding to about 2500 g. of ore, was transferred to a 2000 g. flotation machine. Then 0.15 lb. of sodium sulfide per ton of ore, 0.05 lb. of isopropyl xanthate, and the frother reagent given in Table 3 were added. Air was drawn through the pulp and a concentrate was removed for 10 minutes. The following results were obtained.

As shown in the examples, the froth flotation process is carried out in the following manner:

15 The ore or mineral to be concentrated is first finely ground in the presence of water to the desired size, depending upon the mineral to be treated, to insure that all of the gangue and metalliferous components are liberated from each other. The ground mineral is then screened to remove the oversize materials. The resulting slurry or pulp is transferred to a flotation machine where it is mechanically agitated. The flotation reagents are added to the pulp either in the mill or in the flotation machine depending on the ore that is treated. Water is added to adjust the pulp to the desired solids content. After the reagents have been dissolved or dispersed, air or other suitable gas is passed through the pulp. The desired mineral collects in the froth that is produced on the surface of the pulp and then the froth is removed.

20 The frothing agents used in accordance with this invention are soluble salts of cymene sulfonic acid. The frothing agent may contain 25 considerable amounts of inorganic salts resulting 30 in the concentrate.

Table 3

| Example | Frother Reagent                                    | Lb. per Ton | Lead in Tailings | Lead in Concentrate | Lead Recovery    |
|---------|----------------------------------------------------|-------------|------------------|---------------------|------------------|
| 5.....  | p-Cymene sodium sulfonate (no inorganics).....     | 0.05        | Per cent<br>0.12 | Per cent<br>49.1    | Per cent<br>92.9 |
|         | Hard wood creosote.....                            | 0.15        |                  |                     |                  |
| 6.....  | p-Cymene sodium sulfonate (17-20% inorganics)..... | 0.04        | 0.11             | 54.4                | 94.5             |
|         | Hard wood creosote.....                            | 0.14        |                  |                     |                  |

The p-cymene sodium sulfonate was prepared by a process similar to that in Example 1 except that fuming sulfuric acid was used as the sulfonating agent and the inorganic material was removed by extracting the product with alcohol.

## EXAMPLE 7

A 1020 g. sample of a zinc sulfide ore, which was retained by an 8-mesh screen, was ground on a ball mill for 7 minutes with 1000 cc. of water. The zinc ore was composed of sphalerite, pyrite and a siliceous gangue. The ground ore was screened through a 35-mesh screen and transferred to a 1000 g. flotation machine. The pulp was diluted with water to about 20% solids and conditioned for 10 minutes with 5.5 lbs. of lime per ton of ore and 1.4 lbs. of copper sulfate per ton of ore. Then 0.16 lb. of ethyl xanthate per ton of ore, and 0.22 lb. of p-cymene sodium sulfonate (about 30% inorganics) per ton of ore were added. Air was drawn through the pulp and a concentrate removed for 10 minutes. The tailing contained 0.70% zinc and the concentrate contained 47.0% of zinc. Zinc was recovered in the amount of 96.3%.

From the foregoing examples, it is seen that the present invention provides an improved froth flotation process for separating minerals. The results show a low percentage of metals in

50 from the neutralization of the acid used in preparing the sulfonates. The reagent may contain as high as 60% inorganic salts although with certain ones it is preferable to remove the inorganic salts and use the pure cymene sulfonate. Salts which are suitable include the sodium, potassium, barium and calcium salts of o-, m-, and p-cymene sulfonic acids.

55 The amount of flotation reagent used may vary from about 0.005 to about 5 lbs. per ton of ore, but preferably between 0.01 to 0.5 lb. per ton of ore. The frothers of this invention function over a wide pH range.

60 In most cases, it is necessary to use, along with the frother, other reagents in order to obtain an efficient separation of the mineral. These may be collectors, such as xanthates, mercaptans, organic sulfides, thiophosphates, thiocarbonates, thioureas, thiocarbanilide, azo and diazo compounds; activating and conditioning agents, such as copper sulfate and other salts of copper, lead, zinc, alkali metal sulfides, lime, sodium hydroxide, sodium carbonate, cyanides, 65 alkali metal silicates, etc.; and inhibitors such as glue, starch, gelatin, tannins, etc. Other well known frothers, such as pine oil, cresylic acid, aliphatic alcohols, etc., may be used in combination with the cymene sulfonates.

70 The flotation agents disclosed in accordance

with this invention may be used generally for the dressing of ores including sulfide ores, oxides, non-metallic ores and native metals. Coal may be beneficiated by flotation using the cymene sulfonates. The invention is especially applicable, however, to metallic ores particularly ores containing sulfide minerals of zinc, lead, copper, iron, silver, etc., which may be simple or complex combinations.

Although the applicability of the flotation agent is general for conditioning ores or treating minerals, the conditions effecting the frothing operation are dependent in addition to the froth flotation agent, on the size of the ore being treated, the temperature at which the treatment is being carried out and the per cent solids in the pulp. In each case, the particular conditions may be adjusted so as to permit the flotation agent to perform in an economical and efficient manner.

The cymene sulfonates function as frothers and have practically no collection properties for the minerals; thus, they show excellent selectivity for the mineral over the gangue of the ore. By use of these frothing agents the volume of the froth is easily controlled, the bubbles produced are small, the froth has a long cell life, and the percentage of mineral values in the tailings is low. Only a small amount of gangue is floated and a high grade concentrate is obtained. Since calcium and magnesium cymene sulfonates are soluble, these reagents function efficiently in hard water. Relatively small amounts of a cymene sulfonate are effective in separating the metals from the gangue in an efficient manner, thereby providing an economical method of concentrating ores.

What I claim and desire to protect by Letters Patent is:

1. In the method of concentrating ores, the step which comprises subjecting an aqueous pulp of the ore to froth flotation in the presence of a collector and a water-soluble salt of a cymene sulfonic acid.

2. In the method of concentrating ores, the steps which comprise adding between about 0.005 and about 5 lbs. of a water-soluble salt of a cymene sulfonic acid per ton of ore and a collector to an aqueous pulp of the ore, agitating and aerating said pulp to form a froth containing the desired mineral values of said ore, and separating the said froth.

3. In the method of concentrating ores, the steps which comprise adding between about 0.005 and about 5 lbs. of p-cymene sodium sulfonate

per ton of ore and a collector to an aqueous pulp of the ore, agitating and aerating said pulp to form a froth containing the desired mineral values of said ore, and separating the said froth.

4. In the method of concentrating ores, the steps which comprise adding between about 0.005 and about 5 lbs. of p-cymene calcium sulfonate per ton of ore and a collector to an aqueous pulp of the ore, agitating and aerating said pulp to form a froth containing the desired mineral values of said ore, and separating the said froth.

5. In the method of concentrating a zinc sulfide ore, the steps which comprise adding between about 0.005 and about 5 lbs. of p-cymene sodium sulfonate per ton of ore and a collector to an aqueous pulp of said ore, agitating and aerating said pulp to form a froth containing the desired mineral values of said ore, and separating the said froth.

6. In the method of concentrating a lead sulfide ore, the steps which comprise adding between about 0.005 and about 5 lbs. of p-cymene sodium sulfonate per ton of ore and a collector to an aqueous pulp of said ore, agitating and aerating said pulp to form a froth containing the desired mineral values of said ore, and separating the said froth.

7. In the method of concentrating a copper sulfide ore, the steps which comprise adding between about 0.005 and about 5 lbs. of p-cymene calcium sulfonate per ton of ore and a collector to an aqueous pulp of said ore, agitating and aerating said pulp to form a froth containing the desired mineral values of said ore, and separating the said froth.

WILLIAM T. BISHOP.

#### REFERENCES CITED

The following references are of record in the file of this patent:

#### UNITED STATES PATENTS

| Number    | Name   | Date          |
|-----------|--------|---------------|
| 1,678,311 | Adams  | July 24, 1928 |
| 2,244,512 | Brandt | June 3, 1941  |

#### OTHER REFERENCES

Publication American Institute of Mining and Metallurgical Engineers, Transactions - Milling Methods, "Experiments with Flotation Reagents," by Arthur F. Taggart, T. C. Taylor and C. R. Ince, pages 285 to 368. 1930 edition relied on, page 340 and notes on page 350. (Copy in Div. 26 and Scientific Library.)